

# UNITED STATES PATENT OFFICE.

EDMUND THIELE, OF BRUSSELS, BELGIUM.

## METHOD OF PRODUCING CELLULOSE THREADS.

No. 909,257.

Specification of Letters Patent.

Patented Jan. 12, 1909.

Application filed June 23, 1906. Serial No. 323,071.

*To all whom it may concern:*

Be it known that I, EDMUND THIELE, a citizen of the Empire of Germany, residing at Brussels, in the Kingdom of Belgium, 5 have invented a new and useful Method of Producing Cellulose Threads, of which the following is a specification.

The known method of producing threads from concentrated solutions of cellulose in 10 ammoniacal solution of cupric oxide with the aid of slowly acting precipitants and of subsequently stretching the threads presents the defect, that the threads frequently stick together and therefore furnish a hard, strawy, 15 little bright product. This defect may be obviated by the employment of an alkaline precipitation-liquid, in which the precipitation and the stretching of the threads are effected, so that soft and bright threads are 20 obtained.

My invention relates to a more advantageous method, in which the threads are first precipitated and stretched in a sour or 25 neutral or little alkaline slowly acting precipitation-liquid and are afterwards treated with alkaline baths, more particularly with a caustic lye.

The new method is as follows: A concentrated solution of cellulose in ammoniacal 30 solution of cupric oxide is in a known manner permitted to issue from comparatively wide apertures (of about half a millimeter diameter) into pure water or water with a little acid or alkali. The threads so formed are 35 stretched or drawn out either by rapidly winding them on a roll or by dropping them

through a high head of the precipitation-liquid. Afterwards the threads are drawn through a cold caustic soda of 39° Baumé or through a hot (boiling) lye which is a little 40 less concentrated (but which has a more powerful action than the cold lye) and at last they are treated with acid either at once or during their winding on a drum or after a little time. When hot (boiling) lye is used 45 the resulting threads or fibers show a luster and brilliancy much greater than when cold lye is used.

The method may be varied without departing from the spirit of my invention. 50

I claim:

1. The method of producing cellulose threads, which consists in permitting a concentrated solution of cellulose in ammoniac copper to issue from comparatively wide 55 apertures into a slowly acting precipitation-bath, drawing out the threads so formed in this bath, and subsequently treating them with a boiling caustic lye.

2. The method of producing cellulose 60 threads, which consists in permitting a concentrated solution of cellulose in ammoniac copper to issue from comparatively wide apertures into a diluted caustic lye, drawing 65 out the threads so formed in this bath, and subsequently treating them with a boiling caustic lye.

EDMUND THIELE.

Witnesses:

OTTO KÖNIG,  
ADOLF SCHUBERT.